

## UNITED STATES PATENT OFFICE.

FRIEDRICH W. WEBER, OF HACKENSACK, NEW JERSEY.

## PROCESS FOR TREATING ANIMAL TISSUES AND PRODUCTS OBTAINED THEREFROM.

No Drawing. Application filed March 19, 1925, Serial No. 16,861. Renewed January 31, 1927.

This invention relates to certain products obtained from animal tissue, for instance from animal hides after they have been de-haired and otherwise prepared by any of the well known ways, the object of the invention being to produce a leather of superior whiteness and of unusual lasting properties compared with that prepared by the processes of the prior art; it is also an object of the invention to produce such superior leather also at a low price and with other economical advantages.

The subject-matter of this application is a continuation in part of the original co-pending application, entitled "Method of treating animal tissue and products obtained therefrom", Serial No. 704,282, filed April 4, 1924.

In the present art of tanning the utilization of alum plays a great part though its application entails considerable economical as well as technical disadvantages. One of the causes of these short comings is its high content of water which causes use-less expense for freight and as the alum must be deprived of its iron content before it is applied to the tanning process the originally low priced material has already be-come rather expensive when it is ready for use.

It is also possible that leather produced by a tanning process using alum as a tanning agent will retain sulfuric acid within its intercellular spaces so that it is absorbed by the tissue and in the course of time will act on the leather and will render it brittle; such leather will then easily crumble to pieces on being handled.

Notwithstanding such considerable short-comings alum is applied on a large scale for tanning purposes because it has been found very difficult to find a proper substi-tute for the same. I have found out, as described in my original application referred to above, that the compounds of the rare earth metals readily act as tanning agents as far as the quality of the leather and the cost of its production is concerned. I have also found that the cost of material for the production of a superior leather ac-cording to my process is not higher than that of the processes of the prior art and that it is actually lower in view of the great advantages owing to the saving of time and labor allowed by the great simplicity and unfailing results of my new process.

For the better understanding of my invention I refer to the fact that in the tan-nage with alum a certain amount of sodium chloride is added; practical tanners main-tain that on account of its hygroscopity the sodium chloride in the animal tissue later on softens the same after it has passed the tanning process. On the other side it is claimed that the addition of sodium chlo-ride to the tanning liquor containing alu-minum sulfate causes a double decomposi-tion to take place which results in the forma-tion of  $\text{AlCl}_3 + \text{Na}_2\text{SO}_4$ , of which  $\text{AlCl}_3$  is supposed to act as the real tanning agent. The contentions of both parties are refuted by the experiments of Knapp, (Die Natur und das Wesen der Gerberei-Chemie, 1858; Ueber Gerberei und Leder, Dingler'sches Polytechn. Journal, vol. 181, pg. 311; Rogers, Practical Tanning, 1922, Carey, Baird & Co., New York; Brit. Pat. 2716-1361; D. R. P. 444 and 10,518), said experiments proving that a solution of  $\text{AlCl}_3$  does not act differently upon albumen from a solution of aluminum sulfate and that in both cases the desired coagulate can only be obtained upon the addition of sodium chloride.

While I have described in my original application referred to above that I can produce a leather superior in whiteness and softness to the best French kid leather if I apply one or a plurality of acetates of the rare earth metals, without exception, I have now found out that the situation is not governed by the same generalization if the chlorides of the rare earth metals are con-sidered. I have found that I can produce a leather of excellent whiteness by treating the hides, prepared in the usual way, with a solution of the chlorides of all, or part, or any one of the rare earth metals, pref-erably such as lanthanum, neodymium, di-dymium, praseodymium, ytterbium, yt-trium, with or without the addition of sodium-chloride, the solution, however, to be free of cerium. By extensive emperiments I found that the absence of cerous com-pounds, such as cerium chloride, is nec-es-sary to obtain perfectly satisfactory results as to whiteness and lasting properties. There is no doubt that cerous compounds cause the hide to turn yellow and that the substance of the same is destroyed by the continuous alternate oxidation of the cerous oxide to ceri-oxide and the reduction of the

latter to cerous oxide. These defects are never observed if one treats the pickled hides according to my new process in the presence of sodium chloride with the chlorides of the rare earth metals, but in the absence of cerous chloride,  $CeCl_3$ .

The compounds deposited by the reaction of the aforesaid rare earth metals with the leather are so devoid of acid that they can 10 be considered practically identical with the oxides, or hydroxides, of the rare earth metals in that these compounds are inert to leather. Some of these elements occur in 15 such small quantities that the solution consists more of lanthan and didymchloride than of other chlorides if it is made from the residues obtained from the manufacture of chemicals for the incandescent gas light mantle from monazit sand. Such solutions, 20 however, mixed with sodiumchloride, may be immediately applied for tanning with very satisfactory results for they display a very high power of penetration and tanning effect.

25 I prefer, however, to proceed as follows: The fresh hide, prepared in any of the well known ways, is first treated at approximately 37 deg. C. with a 5% neutral sodium or potassium soap solution. The hide, thus 30 surcharged with soap, is then set up to drain off, or to otherwise remove in any suitable way the mechanically adhering soap, and then it is immersed into the tanning liquor consisting of a solution of a mixture of all, 35 or part, or any of the chlorides, or basic chlorides of the rare earth metals with the exception of cerium, sodium chloride having been added to aforesaid solution. According 40 to the nature of the acid, or acids, contained in the soap, for instance oleic, stearic or palmitic acid etc., the respective salt of the rare earth metals is immediately formed upon the immersion of the hide in the tanning liquor. I wish to state in this regard 45 that the hide should not be impregnated first with the tanning liquor to be subsequently immersed into the soap solution, as the metal salt solution will then run out of the hide to form with the soap a foam on 50 the outside of the hide.

In the process described in the preceding examples I may substitute all the sodium chloride by sodium sulfate and furthermore part of the sodium chloride by zinc sulfate. 55 The hide impregnated with such a tanning liquor containing zinc sulfate is then subsequently acted upon with di-sodiumphosphate whereby the phosphates of the rare earth metals and that of zinc are precipitated within the hide in the form of compounds inert to leather whereby a product 60 of excellent whiteness is obtained.

In this case I can also proceed as follows: The hides, impregnated with the tanning liquor of the chlorides, or basic chlorides,

of aforesaid rare earth metals, free of cerium, but with an addition of zinc sulfate and sodiumchloride, are worked at preferably 37 deg. C. in a drum, or in or by any other suitable mechanical device, with a 70 mixture of egg yolk, flour, sodiumchloride and sodium phosphate, whereby I avoid from the first any loss by the running out of the tanning liquor and secondly I accomplish the double decomposition forming the phosphates of the rare earth metals and zinc under conditions which favor the formation 75 of a jelly from the flour which contributes to yielding a better leather. As all elements combine in the proportion of their atomic weight the quantity of acid radicle in the molecule of the rare earth metal compounds is proportionately smaller than in the compounds of metals of low atomic weight, the amount of acid to produce the 80 neutral salt, or the amount of alkali to turn such a salt into a basic salt, regardless of whether the salt be a sulfate, chloride or acetate, the cost of the materials to perform these changes is smaller than with the other chemicals applied up to now as tanning agents. Moreover, as the compounds coming in consideration for my new tanning process are produced preferably from the residue obtained in the manufacture of the 85 salts for the impregnation of mantles for incandescent gas light, the facts in combination with the favorable circumstances pointed out above makes it self evident that 90 my new tanning process can successfully compete as to economy as well as quality 95 of products with any of the old tanning processes.

Finally I wish to point out that also the 100 leathers produced by this process by means of the chlorides of the rare earth metals are sterile and do not favor the growth of certain micro-organism so destructive to leather. This is important because the sterilization of the hides prevents their destruction by the putrefaction caused by the 105 organic matter, like flesh particles, blood, etc., adhering to the hides; on the other side it is very important that this sterilization 110 be effected with materials which are not 115 detrimental to the hides nor to the people who are using the manufactures made from the sterilized leather. For instance formaldehyde is very effective in preventing putrefaction, but it is highly injurious to the 120 leather as well as to the wearer of the leather product.

I have now found that I can accomplish 125 the sterilization of the hides most satisfactorily in every respect by the action of the rare earth metal salts referred to and applied to the leather by the processes described above. I have especially found that leathers tanned by this process are also distinguished by being proof to mildew; this 130

is strikingly shown by the following test which consisted in moistening leather, having been tanned by any of the above processes, with water and subsequently drying it in an open pan at a temperature slightly above that of the atmosphere, and continuing these operations alternately for 22 weeks without generating even the slightest trace of mildew. It is obvious therefore that leather, obtained by any of the processes, described above, is especially suitable for leather goods intended to be used in tropic climates where the heat and the enormous amount of moisture in the air combine to thoroughly cover goods, made from leather tanned by the processes of the prior art, in a few days with a layer of mildew.

What I claim is:

1. The process of treating hides, comprising acting upon the hides, in the presence of sodium chloride with the solution of a rare earth metal other than cerium.

2. The process of treating hides, comprising acting upon the hides, in the presence of sodium chloride with a plurality of chlorides of the rare earth metals other than cerium.

3. The process of treating animal tissue, comprising acting upon the tissue, prepared in any of the well known ways, first with a solution of a salt, capable of precipitating an insoluble salt from a solution of a chloride of a rare earth metal, and subsequently acting upon the tissue, thus impregnated, with the solution of a chloride of a rare earth metal, other than cerium, in the presence of sodium chloride.

4. The process of treating hides, comprising acting upon the hides, first with a solution of a soap and subsequently acting upon the hides, thus impregnated, in the presence of sodium chloride with a solution of a chloride of a rare earth metal other than cerium.

5. The process of treating hides, comprising acting at approximately 37 deg. C. upon the hides, first with a solution of soap and subsequently acting upon the hides, thus impregnated, in the presence of sodium chloride with the solution of a chloride of a rare earth metal other than cerium.

6. The process of treating hides, comprising acting upon the hides, in the presence

of sodium chloride and zinc sulfate with the solution of a chloride of a rare earth metal other than cerium and subsequently acting upon the hide thus treated with a solution of sodium phosphate.

7. The process of treating hides, comprising acting upon the hides, in the presence of sodium chloride and zinc sulfate with the solution of a plurality of chlorides of rare earth metals, other than cerium, and subsequently acting upon the hides thus treated with a solution of sodium phosphate.

8. The process of treating hides, comprising acting upon the hides, first with a solution of soap and subsequently acting upon the hides in the presence of sodium chloride and zinc sulfate with a chloride of a rare earth metal other than cerium and then acting upon the hide thus treated with a solution of sodium phosphate.

9. The process of treating hides, comprising acting upon the tissue, prepared in any of the well known ways, first with a solution of soap at approximately 37 deg. C., acting upon the hides thus treated, with, in the presence of sodium chloride, a solution of chlorides of rare earth metals other than cerium and then acting upon the hides with a solution of sodium phosphate.

10. The process of sterilizing hides, comprising acting upon the raw hides, from which the flesh particles and other organic matter has been removed, with a solution of soap and subsequently acting upon the hide in the presence of sodium chloride and zinc sulfate with a chloride of a rare earth metal other than cerium and subsequently acting upon the hides thus treated with a solution of a phosphate.

11. As a new article of manufacture, a leather containing in its fibers a deposit of compounds formed by the hide-substance with the aqueous solution of a chloride of a rare earth metal other than cerium.

12. As a new article of manufacture, a leather having in its fibers a deposit of compounds formed by the hide-substance with a chloride of a rare earth metal, other than cerium, in the presence of soap.

In testimony whereof I hereunto affix my signature.

FRIEDRICH W. WEBER.